

## UNITED STATES PATENT OFFICE.

RICHARD LANT, OF VIENNA, AUSTRIA, ASSIGNOR TO WILLIAM KORESKA, OF VIENNA, AUSTRIA.

## STENCIL SHEET.

No Drawing.

Application filed November 16, 1922. Serial No. 601,416.

*To all whom it may concern:*

Be it known that I, RICHARD LANT, chemist, a citizen of the Republic of Austria, residing at 25<sup>a</sup> Gussausstrasse, Vienna, IV, 5 Austria, in the county of Vienna and State of Austria, have invented certain new and useful Improvements in Stencil Sheets, of which the following is a specification.

My invention relates to stencil-sheets of 10 the type commonly used for autographic and typewriting duplication and particularly to stencil-sheets consisting of a fibrous and porous base coated or impregnated with some substance impermeable to the ink, 15 which coating, for the purpose of preparing the stencil, is removed by the pressure of the stylus or by the impact of the types of a typewriter thereon, on the places struck by the type or stylus, so that the ink roller or 20 the like, through these openings liberated from the impermeable substance and forming the letters, can deliver ink to a sheet of paper laid under the stencil. Such stencil-sheets are generally made of open porous material, such as Japanese paper, coated with a wax-like material, such, for example, as paraffin, or with a dry hygroscopic compound of coagulated protein, such as 25 gelatine combined with a suitable tempering agent. The wax-coated sheets have the most disagreeable drawback of being exceedingly brittle, so that in preparing the stencil they are easily injured and that even the finished stencil requires most careful handling. The 30 stencil-sheets coated with coagulated protein are not brittle and offer a considerably greater resistance; besides that the copies made with the latter are sharper and more uniform. But their use is on the other hand 35 more tiresome owing to the circumstance, that in order to adapt the sheet for making the stencil by pressure (as, for instance, by the impact of the types of a typewriter), it is necessary to preliminarily moisten it.

According to the present invention the 40 porous base is coated with a mass including cellulose derivatives, an oil and a normally solid fatty material, the latter for the reason, because it has been found, that it is possible to incorporate a relatively large 45 amount of oil into the mass in order to render the coating supple, if for instance tallow is present in it, whereas without such addition of tallow the stencil sheet is very oily. 50 Moreover, the tallow is adapted for itself to

render the coating more supple and therefore a smaller quantity of the oil is sufficient for obtaining the desired properties. Instead of tallow any other normally solid fatty substance of mineral, vegetable or animal origin may be used, as for instance the fatty acid of cocoanut-oil, paraffine residues and the like. 60

The coating can be made of inorganic or 65 organic esters of cellulose (or of oxy-cellulose or hydro-cellulose) or hydrated cellulose obtained in the manner known per se from solutions of cellulose or cellulose esters by means of a suitable precipitating bath. Furthermore, the coating may include a mixture of esters and of hydrated cellulose, such as is for instance generated 70 when nitro-cellulose is partly denitrated.

The substance or the mixture of substances to be used for the coating is preferably dissolved in a volatile solvent and the coating of the base (porous, fibrous paper sheet) effected by dipping the latter into the solution or by spreading the solution on the sheet by means of a brush or the like. The 75 choice of the solvent depends on the nature of the substance to be dissolved. If, for instance as the normally solid fatty substance to be added to the cellulose ester besides the oil, hydrocarbons or fats are chosen the 80 solvent may be tetrahydronaphthaline (tetraline) or dekahydronaphthaline (dekaline). If for the same purpose fatty acids or substances soluble in a mixture of ethylic ether and alcohol or in amylacetate are chosen, 85 these solvents may be used. In cases where the coating material consists of cellulose esters or the like the solvent is allowed to evaporate after the coating is applied, and the stencil-sheet is then ready for use. To 90 produce a coating which consists wholly or partly of hydrated cellulose, the mass put on the base must be treated thereafter with a suitable precipitating liquid. Thus, for 95 example, a coating made of nitro-cellulose, may be rendered softer as well as more limp and pliable by partly denitrating it.

A practicable formula for use in compounding such a coating (but to which the invention is not limited) is 400 grammes of 100 nitro-cellulose, 800 grammes of castor-oil, 1000 grammes of tallow, 10 litres of amylacetate. To this may be added if desired, a sufficient quantity of a suitable colouring 110 solution.

The stencil-sheets made according to this invention offer the same advantages as the protein-coated sheets in comparison with wax-coated sheets, but are superior to the 5 protein-coated sheets by the fact, that for preparing the stencil they can be used in a perfectly dry state.

I use the term "derivative of cellulose" to include not only one determined derivative, 10 but also a mixture of several derivatives.

What I claim is:

1. A stencil-sheet adapted for stencilization by pressure, comprising a base of open porous material with a type-impressible 15 coating including cellulose derivatives, an oil and tallow.

2. A stencil-sheet adapted for stencilization by pressure, comprising a base of open porous material with a type-impressible 20 coating including cellulose derivatives, castor oil and tallow.

3. A stencil-sheet adapted for stencilization by pressure, comprising a base of open porous material with a type-impressible 25 coating including nitro-cellulose, castor-oil and tallow.

4. A stencil-sheet adapted for stencilization by pressure, comprising a base of open porous material with a type-impressible 30 coating including about 18.18 parts by weight of nitro-cellulose, 36.37 parts by weight of castor-oil and 45.45 parts by weight of tallow.

5. A stencil sheet capable of being stenciled by normal action of the type of a typewriter, or by a stylus, comprising a sheet of 35

open porous material coated with a permanently homogeneous mixture consisting essentially of a cellulose ester, a liquid fatty oil and a normally solid fat, the amounts of 40 said cellulose ester to said liquid fatty oil being such that from a mixture of these two components only, applied to said sheet, separation of oil would occur, and the amount of 45 said solid fat being sufficient to prevent such separation, and being in excess of the amount of liquid oil.

6. A product as covered in the claim last above written, in which the liquid fatty oil is castor oil, and the solid fat is tallow of 50 animal origin.

7. A stencil sheet capable of being stenciled by normal action of the type of a typewriter, or by a stylus, comprising a sheet of open porous material coated with 55 a permanently homogeneous mixture consisting essentially of a cellulose derivative, a greater amount of castor oil and a still greater amount of a hard fat.

8. A stencil sheet capable of being stenciled by normal action of the type of a typewriter, or by a stylus, comprising a sheet of open porous material coated with a permanently homogeneous mixture consisting 60 essentially of about one part of a cellulose ester, about two parts of castor oil and somewhat more than two parts of a hard fat.

In testimony whereof I have affixed my signature.

RICHARD LANT.